

## UNITED STATES PATENT OFFICE

2,092,009

## SAPONIFICATION OF MATERIALS CONSISTING OF OR CONTAINING ORGANIC ESTERS OF CELLULOSE

Robert Wighton Moncrieff, Frank Brentnall Hill, and Thomas Barnard Frearson, Spondon, near Derby, England, assignors to Celanese Corporation of America, a corporation of Delaware

No Drawing. Application December 6, 1934, Serial No. 756,285. In Great Britain December 12, 1933

9 Claims.

(Cl. 8—20)

This invention relates to the treatment of cellulose acetate and other organic esters of cellulose and particularly to a process for reducing the acidyl content of such esters. The invention is specially applicable to the saponification of filaments, threads, yarns, ribbons and the like made of or containing such esters.

It has been discovered that organic esters of cellulose can be saponified by means of non-metallic bases, for example methylamine, ethylene diamine and other aliphatic amines, particularly those of low molecular weight, in the liquid phase with particular advantage, and that by treating threads of cellulose acetate and like materials in this way specially desirable properties may be imparted to the materials. We have now found that the saponification of materials having a basis of cellulose acetate or other organic esters of cellulose by means of non-metallic saponifying agents, and in particular methylamine and similar bases may be accelerated to a remarkable extent by the presence during saponification of copper. The copper is preferably added to the saponifying bath in the form of copper oxide or hydroxide, or a soluble cupric salt, for example copper sulphate. The copper may, however, be applied in other forms. Thus, a marked acceleration of the saponification has been obtained when the copper is initially present in the metallic state.

The organic ester of cellulose treated may be of normal or low viscosity, for example in the case of cellulose acetate the viscosity may be of the order of 30 to 50, 100, 200 or even higher, these figures being obtained by comparison of a 6% solution of the ester in acetone at 25° C. with glycerine at the same temperature taken as a standard of 100. Such esters of high viscosity may readily be made by methods in which degradation of the cellulose molecule is substantially avoided during acidylation, for example the methods of U. S. Patent No. 1,708,787. On the other hand, the viscosity of the cellulose acetate employed may be of the order of 10-20 or even lower, or between 20 and 30, measured on the scale referred to above.

The invention is of particular importance in connection with the saponification of filaments, threads, ribbons, fabrics and like materials having a basis of cellulose acetate and will be described with special reference to the treatment of such materials.

The materials treated may be made by any suitable dry or wet spinning method. Where high tenacity is required in the final products it is of

particular advantage to produce the filaments and the like by wet spinning methods in the course of which they are stretched to a considerable extent, or to soften and stretch the materials after their production whether by a wet or a dry spinning process. By applying the process of the invention to materials which have been stretched considerably, for example to 200% of their original length or even more, materials of particularly valuable serimetric properties are obtainable.

Particularly good results are obtained by the use of saponifying baths containing methylamine and copper. Other strong aliphatic organic bases, for example ethylamine, propylamine, amylamine and triethylamine, may also be employed. Again, somewhat weaker bases of the same series, for example trimethylamine and allylamine, may be used. Further, considerably stronger bases of the same series may be employed, even very strong bases such as tetramethyl ammonium hydroxide, provided care be taken to avoid damaging the materials. Again, amines containing more than one amino group, and particularly aliphatic diamines of relatively low molecular weight, for example ethylene diamine, symmetrical dimethyl ethylene diamine, monomethyl ethylene diamine, and propylene diamine may also be used. Preferably at least one of the amino groups of such amines should be unsubstituted or mono-substituted. Amines containing more than two amino groups may also be employed, for example 1,2,3-triamino propane. The effect of one or more hydroxy groups in the amine appears to be to favour the penetration of the materials by the saponifying agent, and with this object in view substances of the type of  $\alpha$ -diamino- $\beta$ -hydroxy propane may be used with advantage. Again, bases of the heterocyclic series, for example piperidine may be used. Many of these bases appear to enter somewhat readily into combination with copper or copper salts. Some, for instance, readily dissolve copper oxide. The remarkable accelerating effect of copper may perhaps be connected with this phenomenon.

Saponification is preferably effected by subjecting the materials to an aqueous bath containing methylamine or a like acting base and copper in solution. Generally speaking it is advantageous to employ the base in a concentration of 10-30%, and particularly 15-25%. The temperature of the bath may range from below atmospheric temperature to the neighborhood of the boiling point of the solution. It is often convenient to work at temperatures between 15 or

20° C. and 25 or 30° C., but when a high degree of saponification is to be effected it is preferable to work at a somewhat higher temperature, e. g. 50–60° C. or 70° C. or even higher depending on the boiling point of the solution. With a view to preventing excessive evaporation of the base it is of advantage, particularly when working at relatively high temperatures, to cover the surface of the saponifying bath with a layer of an oil, wax or like substance which is immiscible with the bath. The concentrations and temperatures employed in particular cases will naturally depend upon the properties of the particular base employed. In general, the conditions may be chosen so that the desired degree of saponification may be effected by means of a treatment lasting from 1–2 minutes or less up to 3 or 4 minutes. On the other hand the treatment may be more protracted.

20 When the saponifying agent is applied to the materials in the form of an aqueous solution, it is convenient to incorporate the copper, for example in the form of cupric oxide or of a water-soluble salt, for instance copper sulphate, in the 25 saponifying medium itself. It is not, however, essential that the copper should be introduced in this way. It may, for instance, be applied to the materials prior to the application of the saponifying agent, or even introduced into the 30 spinning solution from which they are made.

A very considerable acceleration of the saponifying process may be effected by the presence in the saponifying bath of quite small concentrations of copper, e. g. 0.01–0.05% on the weight 35 of the bath or even less. On the other hand somewhat higher concentrations may be employed, e. g. 0.1% or 0.5%. These figures are based on copper present in the cupric form. Since it is undesirable that the final product should contain substantial quantities of copper it is preferable to work with the smallest quantities 40 capable of giving the desired result.

The saponifying medium may also contain swelling agents, solvents or latent solvents for the cellulose ester, for example cyclohexanol, 45 methyl cyclohexanol, glycerol, ethylene glycol and its mono methyl and dimethyl ethers, diacetone alcohol, benzyl alcohol, acetone, dioxane or methylene ethylene ether.

When the materials are treated in the form of 50 filaments, threads, yarns and the like, it is of advantage to effect saponification "in warp formation", i. e. by drawing a large number of ends through the bath in substantially parallel 55 relationship one to another and in the same plane. Thus, yarn may be drawn from a creel by means of rollers or like devices extending across the entire assembly of ends or so-called "warp" and immersed or partially immersed in a bath containing the saponifying agent, through 60 a reed into the bath, and after passing through the bath the materials may be drawn by a second roller, pair of rolls or the like, situated outside the bath, through a reed and out of the bath, whence they are forwarded to suitable collecting 65 means or to means for effecting any subsequent treatment to be applied. Preferably the materials are washed and dried before being wound.

The saponifying agent may be applied by other 70 means. Thus, for example, the materials in hank form may be suspended from rods which are caused to traverse the length of the bath, and at the same time to rotate so as to expose each portion of the yarn to the same depth in 75 the bath for the same period. Again, the mate-

rials may be treated in the form of bobbins, cheeses or other packages. Any suitable means may in fact be adopted in applying the saponifying agent to the materials. Materials in yarn or like form may be treated continuously with their production and/or with a stretching step. Again, in the case of such materials, stretching may be effected during saponification or, provided saponification has not been carried too far, after saponification. In general it is necessary to soften the materials to enable them to be stretched to the desired extent, and in choosing a suitable softening agent due regard should be had to the extent to which the materials have been saponified.

15 As indicated above, the materials may be saponified in fabric form. This may conveniently be effected by passing the fabric continuously through a bath containing the saponifying agent, for example in an apparatus of the 20 type of the winch dyeing machine.

It is generally advisable to treat the materials after saponification so as to remove any copper remaining therein. Any suitable means may be adopted for this purpose. A convenient 25 means comprises washing the materials with dilute sulphuric acid. Dilute aqueous solutions of other acids may also be employed for this purpose, for example a solution of acetic acid of a concentration about 20% has been found effective.

The materials prior to saponification may be subjected to a treatment adapted to facilitate penetration of the saponification agent. This may comprise the application of water to the 30 materials, or they may be treated with aqueous wetting agents, for example soaps.

The degree of saponification effected may be sufficient to reduce the acidyl content of the ester by 8–10% or even less, but is preferably somewhat higher, for example sufficient to reduce the acidyl content by 20–25% or 30%. Considerably higher degrees of saponification may be effected sufficient to remove 35 or 40 to 50 or 55% of the acidyl content or more, even up to complete 40 saponification, according to the particular purpose in view. Generally speaking, a loss in acidyl content of 20–25 or 30% is capable of rendering the cellulose acetate material insoluble in acetone and imparting to it a high affinity for cotton 45 dyes without destroying the affinity for cellulose ester dyes, for example the so-called S. R. A. dyes. The material may be rendered insoluble in substantially anhydrous acetone but may be soluble in acetone containing a considerable percentage, 50 e. g. 25–30%, of water. Or saponification may render the material insoluble in such mixtures as well as in anhydrous acetone. The saponification may raise the safe ironing point considerably. Materials saponified according to the invention 55 may have, in addition to the valuable properties referred to above, a high tenacity and elasticity and a good extensibility. Such materials are of particular value for use in the manufacture of high twist yarns. Thus, high twist yarns partially saponified according to the invention have been found particularly useful as weft in the manufacture of crepe fabrics. Again, by the process of the invention, it is possible to obtain completely saponified materials of excellent tensile 60 properties.

The following examples illustrate the invention:

#### Example 1

Cellulose acetate yarn is led continuously in

warp formation from a creel through a saponifying bath containing a 15-25% aqueous solution of mono-methylamine to which has been added a sufficient quantity of copper hydroxide to produce a concentration of 0.05 to 0.5% copper. The temperature of the bath is maintained at 25-30° C. and the rate of travel is adjusted so that the yarn is in contact with the bath for 2-3 minutes. In this way a yarn of good tenacity and extensibility having a relatively high safe ironing point and a good affinity for cotton dyes may be obtained with relatively little loss of weight.

*Example 2*

15. The process is carried out as described in Example 1 except that the saponifying bath is maintained at a temperature of 50-60° C. In this way the yarn may be saponified to a considerably greater extent than that treated according to Example 1.

Similarly other non-metallic bases, for example ethylamine, propylamine, ethylene diamine or others of the bases referred to above may be applied.

25. Although the invention has been described with particular reference to the treatment of materials having a basis of cellulose acetate, it is also applicable to the treatment of other materials containing other saponifiable esters of cellulose, for example cellulose formate, propionate, butyrate, ethyl cellulose acetate, oxy-ethyl cellulose acetate and nitrocellulose acetate.

What we claim and desire to secure by Letters Patent is:—

35. 1. Process for reducing the acetyl content of an organic ester of cellulose, which comprises treating the ester, in the presence of copper in solution, with a saponifying agent therefor which is a non-aromatic nitrogenous organic base which contains less than 7 carbon atoms.

2. Process for reducing the acetyl content of an organic ester of cellulose, which comprises treating the ester, in the presence of copper in solution, with a saponifying agent therefor which is a water-soluble nitrogenous base having less than 7 carbon atoms in which each carbon atom that is directly attached to a nitrogen atom is directly attached to three other atoms apart from said nitrogen atom.

40. 3. Process for saponifying filaments, threads, ribbons and like materials having a basis of organic ester of cellulose, which comprises treat-

ing the materials in the presence of copper in solution with an aqueous solution of a saponifying agent therefor which is a non-aromatic nitrogenous organic base which contains less than 7 carbon atoms.

4. Process for saponifying filaments, threads, ribbons and like materials having a basis of an organic ester of cellulose, which comprises treating the materials, in the presence of copper in solution, with an aqueous solution of a saponifying agent therefor which is a water-soluble nitrogenous base having less than 7 carbon atoms in which each carbon atom that is directly attached to a nitrogen atom is directly attached to three other atoms apart from said nitrogen atom.

5. Process for saponifying filaments, threads, ribbons and like materials having a basis of cellulose acetate, which comprises treating the materials in the presence of copper in solution with an aqueous solution of a saponifying agent therefor which is a non-aromatic nitrogenous organic base which contains less than 7 carbon atoms.

6. Process for saponifying filaments, threads, ribbons and like materials having a basis of cellulose acetate, which comprises treating the materials, in the presence of copper in solution, with an aqueous solution of a saponifying agent therefor which is a water-soluble nitrogenous base having less than 7 carbon atoms in which each carbon atom that is directly attached to a nitrogen atom is directly attached to three other atoms apart from said nitrogen atom.

7. Process for saponifying filaments, threads, ribbons and like materials having a basis of cellulose acetate, which comprises treating the materials with an aqueous solution of mono-methylamine in the presence of copper in solution.

8. Process for saponifying filaments, threads, ribbons and like materials having a basis of cellulose acetate, which comprises treating the materials with an aqueous solution of mono-ethylamine in the presence of copper in solution.

9. Process for saponifying filaments, threads, ribbons and like materials having a basis of cellulose acetate, which comprises treating the materials with an aqueous solution of mono-methylamine containing 0.05-0.5% of copper in solution.

ROBERT WIGHTON MONCRIEFF.  
FRANK BRENTNALL HILL.  
THOMAS BARNARD FREARSON.